

Oct. 2, 1945.

C. C. SMITH

2,386,148

METHOD OF TREATING STRAND MATERIALS

Filed Jan. 9, 1943

2 Sheets-Sheet 1



INVENTOR  
C. C. SMITH

BY

ATTORNEY

*J. J. Goodman*

Oct. 2, 1945.

C. C. SMITH

2,386,148

METHOD OF TREATING STRAND MATERIALS

Filed Jan. 9, 1943

2 Sheets-Sheet 2



## UNITED STATES PATENT OFFICE

2,386,148

## METHOD OF TREATING STRAND MATERIALS

Charles C. Smith, Cranford, N. J., assignor to  
 Western Electric Company, Incorporated, New  
 York, N. Y., a corporation of New York

Application January 9, 1943, Serial No. 471,902

3 Claims. (Cl. 117—63)

This invention relates to methods of treating strand materials, more particularly insulated electrical conductors.

In the manufacture of certain types of electrical conductors for use in the communication arts, textile coverings therefor are coated with added insulating material such as cellulose acetate. In such coating processes given lengths of time are required, as well as given temperatures for drying the coating material, and if the length of time and/or temperature should vary excessively or if an excess coating of material should be applied to the conductor, the conductor would be rendered undesirable, possibly not for commercial use, but due to the fact that the coating is rendered opaque and the color of the textile covering is thus indeterminate.

An object of the invention is to provide a method of treating strand materials, particularly electrical conductors coated with insulating materials.

With this and other objects in view, the invention comprises the method which may be practiced to withdraw a strand material from a supply, pass the material successively through a bath of penetrating material and through intermediate wiping elements to allow the penetrating material to penetrate the coating on the strand, the wiping elements serving to remove excess portions of the coating material.

Other objects and advantages will be apparent from the following detailed description when considered in conjunction with the accompanying drawings wherein:

Fig. 1 is a vertical sectional view of the apparatus by the aid of which the method may be practiced;

Fig. 2 is a top plan view of the apparatus, and

Fig. 3 is an enlarged vertical sectional view of a wiping die, this view being taken along the line 3—3 of Fig. 1.

Figure 4 is a fragmentary elevational view of a portion of the improved wire illustrating the relative position of the fabric covering and the transparent coating.

Referring now to the drawings, it will be observed that the apparatus by the aid of which the method may be practiced includes a tank 10 for a supply of liquid 11 which, in the present instance, is a mineral oil, highly purified for the reduction of the moisture content to a minimum, and commercially known as "transil oil" No. 10. Suitable bearings 12 and 14 are mounted upon the side walls of the tank 10 and are adapted to support the ends of a shaft 15, the latter rotat-

5 ably supporting a supply reel 16. A supply of strand material 17 is wound upon the reel, this material, in the present instance, being an electrical conductor 18 with a serving 19 of textile or paper material and an outer coating 20 of cellulose acetate. The material 19 may be of any desired color and if the coating 20 is of a given thickness, and suitably dried, the color of the material 19 will be apparent. However, if the coating 20 is of an undesired thickness, or is 10 rough, or if it has been given an unsatisfactory drying during the process of application, this coating may be rendered opaque, making it difficult, if not impossible, to determine the color 15 of the material 19 which is of great importance in a communication art during the splicing of such cable or the assembling of electrical apparatus in connection therewith.

The present method, therefore, includes the 20 steps of passing the strand material 17 through the bath 11, it being noted that the supply on the reel may also extend beneath the upper surface of the bath. The strand 17 is removed from the supply on the reel in the direction of the 25 arrow (Fig. 1) and passes around a sheave 22, through a spiral wiping element 23, beneath the supply on the reel and into the bath 11, after which it passes around another sheave 24, back beneath the supply on the reel to a third sheave 30 (Fig. 2) identified by reference numeral 25 and from this sheave the strand passes through another spiral wiping element 26, again beneath the supply on the reel and vertically through a final wiping die 27. The sheaves 22 and 25 are mounted upon a common shaft 28, the ends of which are journaled in bearing portions 29 of a bracket 30, the latter being fixed to the tank 10 as shown in Fig. 2. The sheave 24 is mounted upon a shaft 32, the ends of which are journaled in bearing portions 33 of a bracket 34, mounted in the tank 10, as illustrated in Fig. 2. The spiral wiping elements 23 and 26 are identical in structure, having their upper ends pivotally supported at 35 and 36, respectively, in arms 37 supported by the 40 bracket 30. These elements provide a passage-way for the strand material being treated and serve, not only to wipe the excess liquid 11 therefrom, but to remove any excess coating, should 45 such be present.

The wiping die 27 consists of a resilient die member 39 formed of rubber, or any other suitable material, centrally apertured for the passing of the strand material 17 therethrough and supported by a bracket 40 mounted upon any suitable means, not shown, in a position above

the reel and tank as illustrated in Fig. 1. The die member 39 includes a structure indicated generally at 41 for use in mounting the die on the bracket 40.

Considering now the steps of the method, let it be assumed that a full reel with a supply of the material 17 to be treated is mounted on the shaft 15, and the latter disposed in the bearings 12 and 14. The strand material 17 threaded about the sheaves and through the wiping elements and finally through the wiping die 27 may be advanced through the application of a pulling force on the material after it has passed through the die 27. This pulling force, extending longitudinally of the strand, will also be transmitted to the supply reel by the passing of the strand, in its final travel toward the die 27, in engagement with the supply on the reel, thus causing rotation of the reel at a speed desired for the removal of the strand material therefrom. During this advancement of the material, it is withdrawn from the reel, passed into the liquid, advanced through the wiping element 23, after which the material passes through the bath 11 in travelling toward the sheave 24 and again enters the bath in passing beneath the supply toward the sheave 25. The strand material is given another wiping action in the element 26 and is again directed into the bath in passing its final time beneath the supply toward the final wiping step at the wiping die 27. The material 11 of the bath is of a type adapted to penetrate the coating 20, to soften this coating to render it more pliable so that, should there be any excess quantities thereof present, these quantities may be removed by the elements 23 and 25. Furthermore, the material of the bath in penetrating the coating renders the latter transparent so that the material 19 may be readily observed and its color determined.

Thus, through the aid of the apparatus, the method may be practiced to accomplish various results on a single article, namely, a strand of material having a coating which is opaque, or rough, or of an excess size. The strand, or rather the coating thereon, may have any one, two, or all three of these objective features and the

apparatus, without any variations in the structure or the bath, may be employed in successfully carrying out the method steps to remove these objective features. The bath will always be absorbable into the coating, and as a result will render the coating transparent and will also make the coating soft so that any rough spots present may be removed or made smooth and any oversize portions may be reduced. The dies 23 and 26 serve only as wiping dies if the coated strand is of the desired size, but serve as shaping dies during the presence of rough or oversize portions.

Although specific improvements of the invention have been shown and described it will be understood that they are but illustrative and that various modifications may be made therein without departing from the scope and spirit of this invention as defined by the appended claims.

20 I claim:

1. The method of treating a strand of material of a given color having a cellulose acetate coating thereon which has been made undesirably opaque by excess drying thereof, the method comprising passing the coated strand through a bath of mineral oil absorbable into the coating to render the coating desirably transparent, and wiping excess oil of the bath off the strand.

2. The method of treating a strand of material 30 of a given color having a cellulose acetate coating thereon which has been made undesirably rough and opaque by excess drying thereof, the method comprising passing the coated strand through a bath of mineral oil absorbable into the coating to soften the coating and render it transparent, and smoothing the coating.

3. The method of treating a strand of material 40 of a given color having a cellulose acetate coating thereon which has been made undesirably opaque by excess drying thereof, the method comprising advancing the strand longitudinally, directing the strand through a bath of mineral oil absorbable into the coating to render the coating transparent, and wiping excess oil of 45 the bath from the strand.

CHARLES C. SMITH.